

Feb. 25, 1964

G. MANDEL

3,122,488

ELECTRICAL RECORDING MEDIUM

Filed Aug. 22, 1960



Gerald Mandel  
INVENTOR

BY *John V. Hogan*  
ATTORNEY

# United States Patent Office

3,122,488

Patented Feb. 25, 1964

1

3,122,488

## ELECTRICAL RECORDING MEDIUM

Gerald Mandel, Elmhurst, N.Y., assignor to Hogan Faximile Corporation, New York, N.Y., a corporation of Delaware

Filed Aug. 22, 1960, Ser. No. 50,886

9 Claims. (Cl. 204—2)

This invention concerns electrolytic recording and in particular electrolytic recording paper used to transform electrical pulses into graphic recordings and is a continuation-in-part of my application, Serial No. 31,232, filed May 23, 1960, now abandoned.

Electrolytic recording is the art of recording by means of the electrolytic action of an electric current upon a properly sensitized medium. The recording current is localized to produce marks under control of a machine or operator. In facsimile recording it is common practice to scan line-by-line a record sheet with a stylus which carries current modulated according to the instantaneous density of the subject to be reproduced. A properly sensitized sheet, for instance, may be passed under a reciprocating stylus carrying the recording current or the equivalent scanning operation may be carried out in a number of ways well known to those skilled in the art. In order to produce a mark or image on the recording sheet, the sheet must carry on its surface or impregnated in its structure marking compounds which change color or optical density, or both, in response to the passage of an electric current.

Heretofore, in passing an electric current from an anode to a cathode through the paper, it has been generally necessary for the anode to erode to supply metal ions necessary for the formation of a colored mark. In some cases electrolytic recording has been accomplished without the erosion of the electrode as in the marking of azo papers. However, such papers have not been generally successful commercially because of lack of stability thereof. In order for an electrolytic recording paper to be considered stable it should be storable for several months after impregnation, and for several months after recording, and remain substantially unchanged in the color of the background and in the color of the recorded mark.

One of the most successful types of electrolytic recording paper using an eroding anode is that disclosed in U.S. Patent 2,358,839 to Wagner, in which a polyhydroxyphenolic compound is employed in a recording medium. Such a substance, which is normally colorless, has the characteristic of forming a colored complex compound in combination with iron or other heavy metal. The paper is marked between cathode and anode electrodes. The anode which contains the necessary metal required to form the complex compound dissolves into the paper and is gradually consumed during the recording process. This consumption or erosion of the anode has proven disadvantageous since frequent replacement of the anode is required. Heretofore, many attempts have been made to find ways of reducing erosion of the anode without success.

It was discovered quite unexpectedly, according to the present invention, that it would be possible to produce excellent marks in a recording medium marked between cathode and anode electrodes, without the erosion of either of the electrodes, by incorporating a metal-bearing compound and an organic compound in an impregnant medium. The metal-bearing compound is reacted with the oxygen of the air or with an oxidizing agent incorporated in the impregnant and with hydroxide ions ( $\text{OH}^-$ ) electrolytically produced at the cathode

2

to form an intermediate which then reacts with the organic compound to form a colored mark.

An object of the invention is to provide an electrolytic recording paper which is marked upon passage of an electric current therethrough.

Another object is to provide an electrolytic recording paper which contains an organic marking compound together with a metallic salt which reacts with the marking compound only upon passage of an electric current therethrough.

In accordance with the invention, it has been found that an electrolytic recording medium is provided by impregnating paper with compounds which have been heretofore known, but which when used together produce a synergistic effect in that a recorded mark is of greatly improved quality.

One of the compounds is metallic in nature and reacts with hydroxide ions in the presence of an oxidizing agent to form an intermediate higher hydroxide or hydrated oxide which may be colored or colorless. Another of the compounds is an organic material which reacts with the intermediate formed by the first compound to yield an intensely colored mark. Although the recorded mark appears instantly it is believed to be formed from two separate reactions.

The mechanism believed responsible for the first reaction may be understood by considering the reaction which takes place when a cathode and an anode are placed in contact with electrolytic recording paper and a current is passed therethrough. The reaction at the cathode as the water is decomposed is



Hydrogen gas is evolved and hydroxide ions ( $\text{OH}^-$ ) are produced at the cathode.

These hydroxide ions then react with the metallic compound in the presence of the oxygen of the air or with an oxidizing agent incorporated into the impregnant to form an intermediate higher hydroxide or hydrated oxide.

An example of a reaction of this type involving manganese compounds is given below:



where the intermediate is indicated as a hydrated oxide.

The organic compound is then oxidized by the intermediate to yield highly colored products. While it is true that certain of the suitable organic compounds, such as the polyhydroxyphenolics, react with oxygen in the presence of base to yield colored products, the above mentioned reaction with the intermediate generally results in a far more intense mark than could otherwise be obtained.

The mechanism believed responsible for the reaction of the organic compound with the intermediate is believed to be the oxidation of the organic compound to form highly colored compounds having quinoidal structures. An example of a reaction of this type is:



In the case of similar reactions with other organic compounds hereinafter mentioned the reaction products are not precisely known.

The metallic compounds which may be used are those of metals selected from the group consisting of  $\text{Mn}^{II}$ ,  $\text{Co}^{II}$ ,

$\text{Ni}^{\text{II}}$ ,  $\text{Cr}^{\text{III}}$ ,  $\text{Ag}^{\text{I}}$ ,  $\text{Sn}^{\text{II}}$ ,  $\text{Pb}^{\text{II}}$ ,  $\text{Ti}^{\text{IV}}$ ,  $\text{VIII}$ . It should be noted that these metals have a stable lower oxidation state in solution and are capable of being oxidized to a higher intermediate oxidation state in the presence of base produced by electrolysis of water.

The organic compounds which may be used include polyhydroxyphenolic and aromatic polyamine compounds. The polyhydroxyphenolic compounds include gallic acid, catechol, gentisic acid, hydroquinone, and pyrogallol. The aromatic polyamine compounds include o-phenylenediamine, p-phenylenediamine, benzidine and salts thereof, tolidine hydrochloride, and diphenylamine hydrochloride.

Preferred formulations to impregnate about 30 square feet of white porous paper are set out hereinafter. The formulations when impregnated into about 30 square feet of white porous paper will be electrolytically markable upon passage of an electric current therethrough from electrodes applied to the paper. The electrodes need not be consumed in the marking process, and no supplementary heat is required to intensify the mark. The paper will dry out in air after marking, or drying may be accelerated by subjecting it to an air stream or a low-temperature heater bar.

*Example #1*

|                                                                         |    |     |
|-------------------------------------------------------------------------|----|-----|
| $\text{MnCl}_2 \cdot 4 \text{ H}_2\text{O}$                             | g  | 4   |
| $\text{NaCl}$                                                           | g  | 10  |
| $\text{C}_7\text{H}_6\text{O}_5 \cdot \text{H}_2\text{O}$ (gallic acid) | g  | 2   |
| $\text{H}_2\text{O}$                                                    | cc | 100 |
| 5 N NaOH                                                                | cc | 1   |

In the above formulation the manganous chloride can be replaced by manganous sulfate, manganous nitrate or other manganous salts.

*Example #2*

|                                                                         |    |     |
|-------------------------------------------------------------------------|----|-----|
| $\text{NiCl}_2 \cdot 6 \text{ H}_2\text{O}$                             | g  | 4   |
| $\text{NaCl}$                                                           | g  | 10  |
| $\text{C}_7\text{H}_6\text{O}_5 \cdot \text{H}_2\text{O}$ (gallic acid) | g  | 2   |
| 5 N NaOH                                                                | cc | 1   |
| $\text{H}_2\text{O}$                                                    | cc | 100 |

In the above formulation the nickelous chloride can be replaced by nickelous sulfates, nickelous nitrates, or by other nickelous salts.

*Example #3*

|                                                                         |    |     |
|-------------------------------------------------------------------------|----|-----|
| $\text{CoCl}_2 \cdot 6 \text{ H}_2\text{O}$                             | g  | 4   |
| $\text{NaCl}$                                                           | g  | 10  |
| $\text{C}_7\text{H}_6\text{O}_5 \cdot \text{H}_2\text{O}$ (gallic acid) | g  | 2   |
| 5 N NaOH                                                                | cc | 1   |
| $\text{H}_2\text{O}$                                                    | cc | 100 |

In the above formulation the cobaltous chloride can be replaced by cobaltous sulfates, cobaltous nitrates, or by other cobaltous salts.

*Example #4*

|                               |    |     |
|-------------------------------|----|-----|
| Manganese chloride            | g  | 4   |
| Sodium chloride               | g  | 10  |
| Sodium hydroxide (5 N)        | cc | 3.5 |
| Hydrazine sulfate or thiourea | g  | 0.1 |
| Gallic acid                   | g  | 2   |
| Water                         | cc | 100 |

In any of the above formulations, instead of gallic acid, there may be substituted catechol, pyrogallol, or other suitable polyhydroxyphenolic compounds, such as, but not limited to, hydroquinone and gentisic acid, or suitable aromatic amines such as benzidine hydrochloride, tolidine hydrochloride, diphenylamine hydrochloride, o-phenylenediamine, and p-phenylenediamine.

Sodium chloride is used to provide an electrolyte. Other electrolytes may be used alternatively, such as sodium and potassium nitrates and equivalent electrolytes well known in the art.

In the above examples, the quantities given for sodium chloride may vary from zero to 30 grams (the solubility

limit) depending upon the degree of electrical conductivity desired. Similarly, if sodium nitrate is used for an electrolyte, its concentration may vary from zero to 95 grams (the solubility limit).

5 The quantities given for the gallic acid represent the approximate solubility limit for this material. If less than this amount is used the intensity of the resulting mark is decreased.

10 The quantities of the nickelous, cobaltous and manganous salts or combinations thereof used may be varied up to their respective solubility limits.

15 Enough sodium hydroxide is used to produce a final pH of the impregnant solution between 2.5 and 8.5, preferably about 5.0. At lower pH levels the solubility of the polyhydroxyphenolics is depressed while at higher pH values the polyhydroxyphenolics are unstable towards air oxidation. The small concentration of  $\text{OH}^-$  ions produced by the sodium hydroxide has been found insufficient to cause oxidation of the metal ions and 20 darkening of the paper.

25 A recording paper containing organic compounds alone may be subject to discoloration in storage due to oxidation of the organic compound by oxygen in the air. Accordingly, the shelf-life of the paper containing the organic compound may be extended by the addition of stabilizers such as hydrazine or salts thereof, hydroxylamine or salts thereof, or thiourea, to the various formulations. These stabilizers act as oxidation inhibitors for the organic compounds.

30 Typical data is plotted in the curve showing the relationship between optical density and current for formulations in accordance with the teachings herein. Curve 1 shows the density of the mark when manganous chloride is used in the formulation of Example 1 but omitting the gallic acid. Curve 2 shows the density of the mark when gallic acid is used in the formulation of Example 1 but omitting the manganous chloride. Curve 3 shows the density of the mark in the formulation of Example 1. Curve 4, in dashed line, indicates the sum of the ordinates of curves 1 and 2. As stated before, the mark formed when gallic acid and manganous chloride are used together shown by curve 3 is more intense than the sum of the results when either is used alone as shown by curve 4.

35 It is to be understood that, while the term "paper" has been used in this specification, the marking compounds are equally applicable to fabrics or any material of the same general nature which may be suitable for use in electrolytic recording processes. Accordingly, the term "electrolytic recording medium" is to be construed as defining any or all of such materials.

40 While the invention has been described with reference to specific embodiments thereof, it will be understood that other embodiments may be resorted to without departing from the invention. Therefore, the form of the invention set out above should be considered as illustrative and not as limiting the scope of the following claims.

I claim:

45 1. An electrolytic recording medium comprising an impregnated sheet containing as a marking composition a metal compound including a metal selected from the group consisting of  $\text{Mn}^{\text{II}}$ ,  $\text{Co}^{\text{II}}$ ,  $\text{Ni}^{\text{II}}$ ,  $\text{Cr}^{\text{III}}$ ,  $\text{Ag}^{\text{I}}$ ,  $\text{Sn}^{\text{II}}$ ,  $\text{Pb}^{\text{II}}$ ,  $\text{Ti}^{\text{IV}}$ ,  $\text{VIII}$ , said metal being capable of being oxidized to a higher oxidation state in the presence of base, and an organic compound selected from the class consisting of polyhydroxyphenolics and aromatic polyamines which are capable of reacting in an electrically conducting solution with said metal in its higher oxidation state to form colored products.

50 2. An electrolytic recording medium according to claim 1 in which the organic compound is selected from the group of polyhydroxyphenolics and aromatic polyamines consisting of gallic acid, catechol, gentisic acid, hydroquinone, pyrogallol, o-phenylenediamine, p-phenylenediamine,

amine, benzidine and salts thereof, and tolidine hydrochloride.

3. An electrolytic recording medium according to claim 1 in which the pH of the composition is at least 2.5.

4. An electrolytic recording medium according to claim 1 in which the metal compound is selected from the group consisting of manganous salts, nickelous salts, and cobaltous salts.

5. An electrolytic recording medium according to claim 1 in which the organic compound is a polyhydroxyphenolic compound.

6. An electrolytic recording medium according to claim 1 in which a stabilizer is included.

7. An electrolytic recording medium according to claim 1 in which a stabilizer is included and which is selected from the group consisting of thiourea, alkyl derivatives of thiourea, dithiobiuret, hydrazine, salts of hydrazine, hydroxylamine, salts of hydroxylamine.

8. An electrolytic recording medium according to claim 1 in which the metal salt is manganese chloride, the polyhydroxyphenolic compound is gallic acid, a stabilizer is

included for the gallic acid, the composition having a pH of at least 4.5.

9. An electrolytic recording medium according to claim 1 in which the composition consists essentially in approximate parts by relative weight of manganous chloride 1, gallic acid 1, and sodium chloride 5.0.

References Cited in the file of this patent

UNITED STATES PATENTS

|    |           |               |       |                |
|----|-----------|---------------|-------|----------------|
| 10 | 168,466   | Edison        | ----- | Oct. 5, 1875   |
|    | 1,343,978 | Little        | ----- | June 22, 1920  |
|    | 2,082,735 | Heinecke      | ----- | June 1, 1937   |
|    | 2,358,839 | Wagner        | ----- | Sept. 26, 1944 |
|    | 2,430,254 | Solomon       | ----- | Nov. 4, 1947   |
| 15 | 2,570,096 | Calkin        | ----- | Oct. 2, 1951   |
|    | 2,663,656 | Miller et al. | ----- | Dec. 22, 1953  |
|    | 2,776,252 | Schwartz      | ----- | Jan. 1, 1957   |
|    | 2,949,409 | Richards      | ----- | Aug. 16, 1960  |

OTHER REFERENCES

Bureau of Standards Circular C426, Inks, pages 32 and 33, Oct. 16, 1940.